

Oct. 26, 1948.

S. D. WELLS

2,452,533

PREPARATION OF PAPER-MAKING FIBER AND OTHER  
USEFUL MATERIALS FROM STRAW

Filed June 30, 1944



Inventor:  
Sidney D. Wells,

By Board, Pond & Anderson,  
Attorneys:

## UNITED STATES PATENT OFFICE

2,452,533

PREPARATION OF PAPER-MAKING FIBER  
AND OTHER USEFUL MATERIALS FROM  
STRAWSidney D. Wells, Combined Locks, Wis., assignor  
to The Institute of Paper Chemistry, Appleton,  
Wis., a corporation of Wisconsin

Application June 30, 1944, Serial No. 542,987

5 Claims. (Cl. 19—5)

1

This invention relates to the treatment of straw to produce, as the main product of the treatment, a type of fiber which is of special value as a fiber component of paper-making stock. Other objects of the invention are to provide valuable by-products which may be used as stock feed or for other commercial purposes.

This invention is in the nature of an improvement upon the subject matter set forth in my former Patent No. 2,298,994, issued October 13, 1942.

*General method*

Certain types of straw, and particularly flax straw, which result as by-products from a seed crop, contain a substantial percentage of useful fiber. For example, the straw of the flax plant contains a fiber known as bast fiber which is particularly suitable for use in making certain high grade papers and textiles.

Where flax or similar crops are used for the purpose of producing a seed crop, the methods of cultivation and crop treatment are such that it is not ordinarily commercially feasible to make use of the fiber for textile purposes. However, methods of utilizing such straws, for example, as disclosed in my former patent above referred to, have been devised for the purpose of making such fibers available for use in the manufacture of high-grade paper, for instance cigarette paper.

I have discovered that not only is it possible to recover from straws of the type referred to a large percentage of fiber in the form of first-class paper-making material, but also that the other constituents of the straw can be classified into more valuable and less valuable components. For example, the non-fibrous fines, which can be produced as a by-product of my improved process, contain about six per cent of protein and are therefore capable of use as an ingredient of stock or poultry food.

In practicing the improved process, the dry straw is first subjected to a percussive treatment in any suitable type of equipment, for example a rod mill, and the product of such percussive treatment, or preferably so much of the product as will pass through a rather coarse screen of about 2 mesh, or more or less, depending upon the material and conditions, is subjected to a combined screening and pneumatic classification process, the screen employed being rather coarse, for example around 8 mesh, or more or less, depending upon the material and conditions. While the material is passing over the screen, it is acted upon by a counter-current of air of sufficient pressure and volume, so that the

2

lighter particles of fiber and other product of the rod mill are air borne and do not pass through the screen, although of less dimensions than the size of the mesh.

5 In this way, there is screened out from the rod mill product all of the relatively heavy particles of shive or non-fibrous material, but the lighter fiber particles and the finer shive particles or fines are air borne, and therefore not screened out along with the heavy shive parts.

Usually, it is found desirable to subject the material, in its passage over the 8 mesh screen, to considerable agitation so as to effect proper screening. A certain amount of agitation is provided by the action of the material as it passes over the screen, and this action is materially assisted by the counter-current of air passing up through the screen. However, it will ordinarily be found advantageous to employ a screen of the 10 vibrating or gyratory type of which there are many types available for this particular purpose.

15 At this point, it may be stated that I have discovered that, if the rod mill product has been properly treated in the rod mill, so that it will all pass through the openings of a half inch mesh screen, in such material substantially all of the shive particles have been detached from the fiber and, although some fiber particles or bunches may be of a size which will not pass 20 through an 8 mesh screen, on the other hand, practically all of the shive is in particles less than 25 8 mesh in size. In other words, the rod mill treatment effects a substantially complete separation between the fiber and the shive leaving 30 most of the shive in condition to pass through the 35 8 mesh screen.

However, the rod mill treatment also produces some small portions of fiber and small shive portions of various sizes collectively designated as 40 fines, all of which are capable of passing the 8 mesh screen; the counter current of air provided at the screen prevents the loss of these fine particles at the 8 mesh screen, and in addition accomplishes the agitation function previously 45 described. Therefore, the material which passes beyond the 8 mesh screen is found to consist substantially of fiber particles or bunches of various sizes together with an admixture of shive particles of sizes below about 40 mesh. This air borne 50 mixture also contains a considerable percentage of dust-like material of extremely fine mesh.

The screened mixture of fiber, fines and finer dust is then subjected to a further separation on a 40 mesh screen, which serves to screen out the 55 non-fibrous material, leaving the fiber on the

top of the screen. This fiber which results as the main product of the process is used for paper-making in the same manner as the fiber produced in accordance with my prior Patent No. 2,298,994. Additional intermediate separations and classifications are within the contemplation of the invention, as will hereinafter appear, but the foregoing outlines the basic steps of the separation process of the invention.

It will be seen, therefore, that the products of the process consist of fiber, coarse shive and fines, the dust being usually considered a part of the fines. Although in certain instances, under certain conditions, it may be possible to separate the fines from the rod mill product prior to the separation of the coarse shive particles, it is advisable to postpone this step until after the coarse shive has been removed, as above described.

*Specific example*

In applying the invention to the treatment of the straw resulting from the production of a crop of flax seeds, it is desirable to use an apparatus of the general stype disclosed in the drawing accompanying this application.

Referring to the drawings, 1 represents a conventional type of rod mill in which the percussive treatment is effected. Said rod mill is fed with flax straw by a suitable feeder such as a screw conveyor 2, which receives the raw material through the hopper 3. For reasons of economy and production of a high-grade product, it is not advisable to carry the percussive treatment in the rod mill to such an extent as to complete the percussive treatment on 100% of the material, and therefore it is preferred not to equip the rod mill with a screen, but to use a screen on the discharge, and return the over-size to the inlet of the rod mill for further treatment. This is done by permitting the material discharged from the rod mill to feed rather freely into the discharge hood 4 at the lower end of which is an opening 5 to an enclosed chute 6 equipped with a pair of gyratory screens 7 and 8. The upper screen may be of approximately 2 mesh, while the lower screen is of about 8 mesh. It may be assumed that any product which is not capable of passing through the 2 mesh screen probably includes the fiber and shive components which have not been sufficiently worked in the rod mill to fracture the bond between the shive and the fiber, and therefore these larger particles are allowed to pass on to a spout 9 equipped with a suitable air seal 10 and fall onto the upper stretch 11 of a belt conveyor. These over-size particles of rod mill product are then delivered to the boot 12 of an elevator 13, and delivered from the elevator spout 14 into the feed hopper 3 previously referred to. In this manner, the oversized particles are re-cycled for re-treatment.

The selected product which passes through the 2 mesh screen drops onto the lower 8 mesh screen, and the heavy or coarse shive parts pass through the 8 mesh screen into a funnel 15 reaching into the top of a closed bin 16. In the top wall of said bin there is inserted a pipe 17 by means of which air may enter the bin 16. However, the flow of air through pipe 17 may be regulated by a damper 18.

That portion of the chute 6 which is located between the 2 mesh and the 8 mesh screen, at its lower end communicates freely with a discharge pipe 19 which, in turn, is connected to the lower end of an up-take pipe 20. By means, later to

be described, pipe 20 is subjected to an upward suction, and hence there will be an up-draft of air through the 8 mesh screen 8, the control of said suction being effected by damper 18. Hence only the coarse shive parts will pass through the screen 8, the remainder of the material consisting of fiber and shive fines being saved and sucked upward through pipe 20.

The pipe 20, at its upper end, discharges tangentially into the upper or large diameter portion of a cone classifier or cyclone 21, the vent or discharge 22 of which is connected into the eye of a centrifugal fan 23. Said fan constitutes the means for subjecting the uptake pipe 20 to the required suction. In certain instances, it may be advisable to connect the upper end of the hood 4 directly with the upper portion of pipe 20 by means of a by-pass 24 controlled by a suitable damper 25. By this means, it is possible to provide a short cut path of movement for the extremely fine particles such as dust or other light material which go direct to the classifier or cyclone 21 without having to pass through the chute 6 and up pipe 20. The amount of said by-pass effect can, of course, be regulated by adjustment of the damper 25.

The discharge 26 from the bottom of the cyclone or classifier 21 enters a chute 27 within which there is located a 40 mesh shaking or gyratory screen 28, this screen being of substantially the correct mesh to screen out the desired fiber from the material discharged from the classifier 21.

That part of the chute 27 which is located above the 40 mesh screen is connected to a discharge duct 29 which enters the closed fiber bin 30, in which the fiber is accumulated and withdrawn from time to time. That part of the chute 27 which is below the 40 mesh screen 28 leads 40 into a separate discharge pipe 31 leading into a closed bin 32 for receiving the shive fines.

In certain cases, it may be feasible to lead the discharge 33 of the exhaust fan 23 directly into the atmosphere. However, on account of the fact that it may be advisable to save the powder-like fines as well as the fines of larger size, it is preferred to connect said discharge 33 to another cyclone 34 of the collector type. Said collector cyclone 34 has its vent 35 connected directly to the atmosphere, while the lower end of the cone of the cyclone collector is connected to a pipe 36 which communicates with the fines bin 32 through a suitable air seal 37.

I claim:

1. The improved method of obtaining a selected useful fiber from a flax straw which comprises the steps of fracturing the bond between the straw fiber and shive so as to produce a mixture of relatively large particles of shive, relatively smaller and lighter particles of shive, the selected fiber in various lengths, and dust, separating the large particles of shive from the selected fiber and the other constituents of the said mixture by passing the mixture over a screen while subjecting the mixture to a counter current of air of such intensity that the large particles of shive are able to pass through the screen by gravity, whereas the fine particles of fiber, the fine shive particles, and the dust are restrained from passing through the screen, and subsequently separating the selected fiber from the material which is restrained from passing through said screen by a process which includes a second screening operation.
2. The improved method of obtaining a se-

lected useful fiber from a flax straw which comprises the steps of fracturing the bond between the straw fiber and shive so as to produce a mixture of relatively large particles of shive, relatively smaller and lighter particles of shive, the selected fiber in various lengths, and dust, separating the large particles of shive from the selected fiber and the other constituents of the said mixture, by passing the mixture over a mechanically agitated screen while subjecting the mixture to a counter current of air of such intensity that the large particles of shive are able to pass through the screen by gravity whereas the fine particles of shive, the fine particles of fiber, and the dust are restrained from passing through the screen, and subsequently separating the selected fiber from the material which is restrained from passing through said screen by a second screening operation involving the use of a second mechanically agitated screen having a sufficiently fine mesh to screen out the desired fiber.

3. The improved method of obtaining bast fiber from flax straw, which comprises the steps of percussively treating said flax straw to fracture the bond between the bast fiber and the straw shive so as to produce a mixture of relatively large particles of shive, relatively smaller and lighter particles of shive, the desired bast fiber in various lengths, and dust, separating the large particles of shive from the bast fiber and the other constituents of said mixture by passing the mixture over a mechanically agitated screen of about 8 mesh while subjecting the mixture to a counter current of air of such intensity that the large particles of shive are able to pass through the screen by gravity, whereas the fine particles of bast fiber, the fine shive particles, and the dust are restrained from passing through the screen, subsequently effecting further separation by pneumatic means of the bast fiber from the mixture which is restrained from passing through said screen, and finally effecting substantially complete separation of the bast fiber from the material resulting from the pneumatic separation by the use of a second mechanically agitated screen, this screen being of about 40 mesh.

4. The method of separating bast fiber from flax straw, which comprises the steps of first passing the straw through a percussive zone so as to convert the straw into a decorticated mixture which includes relatively light particles of fiber, relatively large particles of shive and straw, relatively smaller particles of shive, and dust, providing a zone of low pressure adjacent said percussive zone for drawing said decorticated mixture from said percussive zone as said straw is broken up, continuously withdrawing air, relatively light particles of fiber and dust from the top of said zone of low pressure and conducting the same to a pneumatic separating zone, continuously withdrawing the remainder of said decorticated mixture by gravity from the bottom of said zone of low pressure, the material which is withdrawn from the bottom of said zone of low pressure being conducted in sequence through a first screening zone, which includes a coarse mesh screen, and a second screening zone in which said material is passed across a screen of

substantially finer mesh while being subjected to a countercurrent of air of such intensity that the large particles of shive pass through said screen by gravity to a discharge point, while relatively light particles of fiber, relatively smaller particles of shive and dust are conducted to said pneumatic separating zone, the material retained on said coarse mesh screen being recycled to said percussive zone, and finally separating said bast fibers from the material retained in said pneumatic separating zone by first withdrawing the dust and then passing the remaining material over a screen of fine mesh to separate the bast fibers from the relatively smaller particles of shive.

5. The method of separating bast fiber from flax straw, which comprises the steps of first passing the straw through a percussive zone so as to convert the straw into a decorticated mixture which includes relatively light particles of fiber, relatively large particles of shive and straw, relatively smaller particles of shive, and dust, providing a zone of low pressure adjacent said percussive zone for drawing said decorticated mixture from said percussive zone as said straw is broken up, continuously withdrawing air, relatively light particles of fiber and dust from the top of said zone of low pressure and conducting the same to a pneumatic separating zone, continuously withdrawing the remainder of said decorticated mixture by gravity from the bottom of said zone of low pressure, the material which is withdrawn from the bottom of said zone of low pressure being conducted in sequence through a first screening zone, which includes a mechanically agitated screen of about 2 mesh, and a second screening zone in which said material is passed across a mechanically agitated screen of about 8 mesh while being subjected to a counter current of air of such intensity that the large particles of shive pass through said screen by gravity to a discharge point, while relatively light particles of fiber, relatively smaller particles of shive and dust are conducted to said pneumatic separating zone, the material retained on said 2 mesh screen being recycled to said percussive zone, and finally separating said bast fibers from the material retained in said pneumatic separating zone by withdrawing the dust and passing the remaining material over a mechanically agitated screen of about 40 mesh to remove the relatively smaller particles of shive.

SIDNEY D. WELLS.

## REFERENCES CITED

The following references are of record in the file of this patent:

## UNITED STATES PATENTS

| Number    | Name                  | Date          |
|-----------|-----------------------|---------------|
| 372,016   | Davis, Jr. -----      | Oct. 25, 1887 |
| 869,742   | Slade et al. -----    | Oct. 29, 1907 |
| 1,293,444 | Hubler -----          | Feb. 4, 1919  |
| 1,484,208 | Davis -----           | Feb. 19, 1924 |
| 2,239,059 | Schwartz et al. ----- | Apr. 22, 1941 |
| 2,280,903 | Ellison -----         | Apr. 28, 1942 |
| 2,298,994 | Wells -----           | Oct. 13, 1942 |